

## UNITED STATES PATENT OFFICE

2,040,881

METHOD FOR ELECTROLYTIC DEPOSITION  
OF CHROMIUMFlorice A. Rojas, New York, N. Y., assignor to  
Rojas Chemical Works, Inc., New York, N. Y.,  
a corporation of New YorkNo Drawing. Application May 15, 1931,  
Serial No. 537,745

3 Claims. (Cl. 204—1)

This invention relates to the electrolytic deposition of chromium, as well as the methods and means employed in connection therewith.

The object of this invention is to provide methods and means for chromium plating which offer decided advantages in efficiency, flexibility and economy over the methods heretofore suggested or used.

A further object of the invention is to improve the art of chromium electroplating by making use of the advantages which are inherent to the principles of secondary deposition. Among these advantages are fine grained deposit; maximum throwing power; maximum distribution of the deposit; maximum range of current density and current quantity in bright plating; the elimination of critical values in the physical and chemical characteristics of the bath, such as temperature and chemical balance.

20 A further advantage of my invention is that it permits the electroplating of chromium directly on the metals of which the objects to be plated are made without preliminary coating with copper and nickel as is customary at the present time.

25 A further advantage of my invention is the ability of rendering heavy deposits of chromium either by the use of high current density without limitation of time, when hard deposits are desired; or low current density also without limitation of time when soft and ductile deposits are desired.

A further object of the invention is to provide such an electrolyte for use in connection with the electrolytic deposition of chromium as will be capable of rendering any of the foregoing results commercially practical.

Further objects of the invention will appear more fully hereinafter.

The invention consists in the method of electroplating, as well as the electrolyte employed in connection therewith, all as will be more fully hereinafter set forth and finally pointed out in the appended claims.

In the chromium electroplating processes heretofore proposed or utilized, the principles of primary deposition have been employed notwithstanding the decided advantages that would be obtained by utilizing secondary deposition methods.

50 Primary deposition refers particularly to the electroplating of metals directly from the first ionization of the electrolyte. It is limited to the plating out of two substances, one of them being always hydrogen and the other the metal which is intended to be deposited.

Secondary deposition, however, refers to the electroplating of metals by a subsequent ionization of the anodic ions created by the first ionization of the electrolyte. It involves the plating out of more than two substances, plating out (besides hydrogen and the metal in question) a third metal which I will hereinafter refer to as a Katholyst.

For the sake of conciseness, the word Katholyst will be used throughout this discourse to signify such element or substance which, when forming part of an electrolyte, will, by the passage of the current, separate at the cathode, but will neither remain nor there maintain its chemical and physical constitution without reacting rapidly with the electrolyte.

A Katholyst may be further defined as being such a substance which is readily reduced cathodically to a chemically active condition. In this state it is a powerful chemical reducing agent which reacts rapidly with the depolarizer present, becoming thus reoxidized into a chemically passive condition in the process, from which state it is again cathodically reactivated, and the cycle continues.

In the ionization of a solution of a double salt of a Katholyst and the metal to be plated, the Katholyst forms the positive ions and the acid salt of the metal forms the negative ions. The Katholyst separated at the cathode immediately reacts with the electrolyte to form a hydroxide and thus reestablishes the negative charge of the cathode. The negative ion of the ionization equilibria, on account of its metallic component, is in itself an unstable compound. As soon as the negative charge of the cathode is reestablished by oxidation of the Katholyst, the metallic component of the anion becomes positive, migrates to the cathode and, discharging its positive electricity, neutralizes the negative charge of that electrode, and plates itself there as a metal.

In all the electrolytic processes of secondary deposition in use at the present time, that is, the internal electro-chemical reactions between a metal and the Katholyst, such substances as potassium, sodium, ammonium and the related elements and compounds have been used as the Katholyst. Examples of these processes are the electro deposition of silver from the double cyanide of silver and potassium; the electro deposition of copper from the double cyanide of copper and sodium and the electro deposition of nickel from the double sulphate of nickel and ammonium.

The chemical characteristics of chromium, on

account of the double nature of this metal, differ basically from those of silver, copper and all the noble and semi-noble metals. Chromium partakes of both of the properties of the metals and the non-metal elements in that it is capable of forming either a base or an acid radical. With chromium, salts are formed such as sodium chromate, or chromium sulphate. In the first instance, chromium supplies an acid and, in the second, it supplies a base. Such chemical propensity is not the behavior of true metals in the strict sense of the term.

Due to this double nature, chromium is capable of forming either positive or negative ions. The 15 passage of the current through a solution of chromium sulphate for instance, will discharge the positive electricity of the cathions and precipitate free atoms at the negative electrode. In a solution of sodium chromate, however, chromium 20 will form negative ions, and consequently no direct deposit of metallic chromium will result from this electrolyte.

The use of such complex electrolytes such as the solutions either of the double chromate of 25 sodium and chromium or the double chromate of potassium and chromium containing free chromic acid, will, while complying with the principles of secondary deposition, fail to give the desired results. In the presence of such strong bases as 30 those of the alkaline metals, the chromium ions will be destined to carry the negative charges of electricity.

This behavior of chromium in the presence of 35 the alkaline bases probably accounts for the fact that for the electro deposition of chromium the principles of secondary deposition have not, to my knowledge, been heretofore utilized.

It is among the special purposes of my present invention to overcome the disadvantages and limitations imposed by primary deposition methods 40 with respect to chromium plating and to obtain the advantages inherent to the principle of secondary deposition for electroplating of chromium. This I am enabled to do after extensive 45 experiments extending over a considerable period of time by finding a material to be used as a Katholyst heretofore unused as such in connection with chromium plating or any other metal deposition.

50 I have discovered that when aluminum in any chemical form, but more particularly gelatinous hydroxide, is used in the construction of an electrolyte intended for chromium plating it affords a marked improvement over the use of any addition agent and will deposit chromium even in the presence of the very strong bases of the alkaline metals in the electrolyte.

One noteworthy advantage that this new electrolyte has over those using sulphuric acid as an 60 addition agent, is the inexhaustibility of the aluminum in its Katholistic action.

65 Aluminum, in its Katholytic cycle as above stated, constantly changes its chemical constitution but does not change its quantity. In sulphate electrolytes, however, the sulphuric acid forms the anions and is constantly being exhausted by its chemical combination with the anode. It is evident, therefore, that the new electrolyte 70 using aluminum for its operation will not require the professional skill and constant attention that the sulphate bath does for the maintenance of its working conditions.

75 It is a requisite, for the best results, in the construction of the Katholistic chromium bath to

have no other inorganic acid present in the electrolyte other than chromic acid.

Were there to be introduced sulphuric acid besides the aluminum Katholyst some complications would arise in the ionization of a number of distinct salts of both the chromic and sulphuric acids and aluminum oxides and chromous oxides as the bases, resulting in erratic performance of the bath. It is, therefore, desirable to keep the Katholistic chromium bath free from any other 10 inorganic acid.

Organic acids or other suitable organic substances in the presence of the strong oxidizing power of chromic acid will be changed into carbonic acid and water and the consequent formation of trivalent chromium.

As above stated, the electrolytes for chromium plating in general employ acid radicals as addition agents. These addition agents promote the electrolysis of water having the hydrogen ions 20 wastefully diverting a great percentage of the current at the sacrifice of current efficiency in the deposition of the chromium metal. Furthermore, this effect is prolific of negative conditions 25 in chromium plating and explains to a great extent the instability of operation, narrow range of current density, low current efficiency, critical working points, and many other of the undesirable results which render chromium plating by means of the processes now employed an arduous and 30 expensive task.

It is well known that in electroplating fine grained deposits of metals, maximum covering power and great range of current densities are proportional to the complex chemical composition of the electrolytic bath. This is due to the fact that in electrolytes having complex ions the metal ion concentration is very low. Low metal ion concentration such as would occur in highly dilute solutions however is not sufficient in itself 40 to insure an efficient deposit. The passage of the current will soon remove the metal ions which are present and there is insufficient metal available to be discharged. An inferior, burned and spongy deposit is the result. Therefore, means 45 must be provided to obtain such an amount of dissolved metal salts as will furnish a sufficient supply of ions nearly as fast as they are removed.

I have succeeded in depositing chromium by 50 secondary deposition using a solution of a double chromate of chromium and aluminum and using free chromic acid as a means of maintaining the proper pH of the electrolyte.

As an example of the electrolyte employed, to one gallon of water is added from 16 to 54 ounces 55 of chromic acid ( $\text{CrO}_3$ ) and from 5 to 15% of gelatinous aluminum hydroxide by weight of chromic acid. Upon electrolysis for a period of time, I have found that the electrolyte becomes more and more efficient and the quality 60 of electroplating improved. I have, therefore, found that by supplying salts or solution of the following constituents—



65 an electrolyte may be obtained which initially, as well as throughout its life, will give the desired results.

With the electrolyte thus produced the actual metal cation concentration is very small and 70 the amount of metal salt dissolved in the solution is very large. Thus, fine grained deposits are obtained because, under the influence of a high current, the rapid growth of each crystal of metal is prevented from the scarcity of metal 75.

cations and a greater number of small crystals is the result. However, by changing the current density, i. e. lowering it, in the electrolyte and in accordance with the process of my invention, 5 a softer and coarser grain deposit is obtained.

Maximum distribution of the deposit obtained in accordance with my invention through utilizing maximum throwing power in complex cation solutions is explained by the phenomenon of polarization. While I advance such explanation 10 I desire to have it understood that I do not desire to be limited or confined thereto, as such explanation is advanced as a theory for what benefit it may be. Complex electrolytes, on account 15 of their low cation concentration, offer a marked resistance to the passage of the current to those points of the cathode which are nearer to the anode. At those points polarization is greater because of their comparatively greater proximity 20 to the anode. These nearer points are exposed to higher current densities than the far points of an irregular cathode surface and the discharge of the cations at the near point is faster than the supply from the dissolved metal salts in their 25 vicinity. This propensity has a tendency to equalize the distribution of the secondary current and consequently produces a more uniform thickness of distribution of the deposit upon the entire contour of the irregular cathode surface. 30

It is evident from the foregoing that a greater range of current density is possible in plating from complex or low cation concentration than from simple or high cation concentration solutions. In the complex cation of electrolytes 35 designed for secondary deposition the unretained cation or Katholysts, according to accepted theory, will plate out ahead of the metal which it is intended to obtain, and consequently the cathode efficiency decreases as the current density increases. This automatic check on the 40 deposit of the desired metal on the high points permits the use of a greater range of current densities in secondary than in primary depositions. Hence, in accordance with my invention, 45 the range of current densities is extremely wide

in chromium plating, whereas in processes heretofore employed it is confined to a narrow range of current density. Obviously, as a result, I am able to control at will the physical characteristics insofar as finish, grain, etc., of the chromium deposit. 5

While I have confined my discussion hereinbefore to complex ions in electroplating incident to secondary deposition, it will be readily apparent that the same principles will apply to 10 tertiary deposition, etc. I have in fact obtained chromium plates having a special texture by tertiary deposition from the three chromates of sodium, aluminum and chromium, and also by the tertiary deposition of the tetra chromates 15 of potassium, sodium, aluminum and chromium. Therefore my invention is, broadly stated, directed to the utilization of complex ion electroplating, as distinguished from the primary deposition methods heretofore long found and 20 thought alone to be of commercial utility.

Having now set forth the objects and nature of my invention and having described the details thereof and the formulæ incident thereto, what I claim as new and useful and desire 25 to secure by Letters Patent is:

1. A chromium plating bath containing chromic acid but devoid of other inorganic acids and consisting essentially of a water solution of the 30 oxides of chromium and aluminum.

2. A bath for the electrodeposition of metallic chromium consisting essentially of a water solution of chromic acid free from other inorganic acids and containing from 16 to 54 ounces of chromic acid ( $CrO_3$ ) per gallon of water and 35 from 5 to 15 per cent by weight, based on the weight of the chromic acid, of aluminum hydroxide dissolved therein.

3. The method of electrodepositing metallic chromium which comprises electrolyzing a bath 40 consisting of a water solution of chromic acid free from other inorganic acids and having aluminum hydroxide dissolved therein.

FLORICEL A. ROJAS.

45